

# United States Patent

[11] 3,607,790

[72] Inventor **John J. Pitha**  
Lenox, Mass.  
[21] Appl. No. **781,473**  
[22] Filed **Dec. 5, 1968**  
[45] Patented **Sept. 21, 1971**  
[73] Assignee **General Electric Company**

[56] **References Cited**  
UNITED STATES PATENTS  
3,291,759 12/1966 Pitha ..... 252/516  
3,480,452 11/1969 Fleischner ..... 106/39

*Primary Examiner*—Douglas J. Drummond  
*Attorneys*—Sidney Greenberg, Francis X. Doyle, Vale P. Myles and Frank Neuhauser

[54] **RESISTANCE MATERIAL AND METHOD OF  
MAKING**  
9 Claims, 1 Drawing Fig.

[52] **U.S. Cl.** ..... **252/516**,  
252/521, 106/39, 106/44  
[51] **Int. Cl.** ..... **H01b 1/04**,  
C04b 35/14  
[50] **Field of Search** ..... **252/516,**  
521; 106/39 DV, 44

**ABSTRACT:** Lightning-arrester resistance material is composed of silicon carbide particles and a binder therefor composed of cordierite formed of a fired mixture of cordierite-forming glass material and cordierite-forming crystalline material.



PATENTED SEP 21 1971

3,607,790



Inventor,  
John J. Pitha,  
by Sidney Greenberg  
His Attorney.

## RESISTANCE MATERIAL AND METHOD OF MAKING

The present invention relates to resistance material, and more particularly to resistance material for use with electric discharge devices, such as lightning arresters, and the method of making the resistance material. Such material, also known as nonlinear resistance or valve element material, is of the type having variable resistance characteristics, so that when placed in electrical circuit with a source of electrical potential applied thereto, its resistance decreases with an increase in the electrical potential. In known types of overvoltage protective devices such as lightning arresters, a gap structure is usually arranged in series with the resistance material, and when the device is subjected to overvoltage, such as caused by lightning or a switching surge, the gap arcs over and with the nonlinear resistance material forms a low-resistance path to ground. The resistance material provides a low-resistance path to high voltages and a high-resistance path to low voltages. When the overvoltage surge has been discharged, the resistance material provides a high-resistance path to the the power follow current, limiting such current to enable the gap structure to interrupt the current and return the arrester to its open-circuit condition.

Resistance material of the above-described type comprising a mixture of silicon carbide particles and a binder material therefor comprising cordierite is disclosed in U.S. Pat. No. 3,291,759—Pitha, granted Dec. 13, 1966. The present invention is an improvement on the material and method of the latter patent.

It is an object of the invention to provide improved nonlinear resistance material of the above-described type and a method of making the same.

Another object of the invention is to provide non linear resistance material of the above type having improved resistivity conditions while providing reduced power follow currents.

A particular object of the invention is the provision of an improved non linear resistance material comprising silicon carbide particles and a cordierite binder therefor.

Still another object of the invention is to provide an improved composition and method for forming cordierite, and for making nonlinear resistance material incorporating such cordierite-forming composition.

Other objects and advantages will become apparent from the following description and the appended claims.

With the above objects in view, the present invention in one of its aspects relates to a method of making nonlinear resistance material comprising the steps of mixing silicon carbide particles with a cordierite-forming glass material and cordierite-forming crystalline material, compacting the mixture, and firing the thus-treated mixture at elevated temperature for reacting the crystalline material and for forming a cordierite binder for the silicon carbide particles from the mixture of glass material and crystalline material.

The invention will be better understood from the following description taken in conjunction with the accompanying drawing, in which:

The single FIGURE is a graph showing a comparison of the volt-ampere characteristics of the resistance material of the present invention and those of prior art resistance material.

In the aforementioned Pitha patent, there is disclosed a nonlinear resistance material formed of a mixture of silicon carbide particles and a cordierite binder therefor, wherein the binder material is obtained by firing a mixture of appropriate proportions of talc and a porcelain mixture including flint, clay and soda or potash spar.

In accordance with the present invention an improved resistance material is made by including in the initial binder mixture a suitable proportion of cordierite-forming glass. By "cordierite-forming glass" as used herein is meant a noncrystalline solid material having the composition  $2\text{MgO} \cdot 2\text{Al}_2\text{O}_3 \cdot 5\text{SiO}_2$  and which when heated to elevated temperature below the melting point of the glass and gradually cooled will form a ceramic composed of cordierite. The cordierite-forming glass

used in the present invention (also referred to herein simply as cordierite glass) is thus distinguished from the aforementioned mixture of crystalline compounds used in the prior process to form the cordierite binder in the fired product. As indicated, however, both types of cordierite-forming materials are used in the present invention to obtain nonlinear resistance material of optimum properties.

By virtue of the addition of cordierite glass to the binder-forming material in accordance with the invention, the resultant resistance material retains all the advantages of the prior material made with only crystalline cordierite-forming compounds, such as low resistivity to overvoltages and high capacity to withstand repeated surges of current, and in addition it is characterized by a substantially higher resistance in the low voltage range than the prior resistance material. As a result, the improved material when used, for example, in lightning arresters, more effectively cuts out power follow currents and thus enables more rapid extinguishing of the arc formed by overvoltages in the arrester, so that the electrical apparatus protected by the arrester resumes normal operation in a shorter time. An additional advantage obtained by such properties of the non linear resistance material is that the life of the lightning arrester is thereby substantially prolonged.

The FIGURE graphically illustrates the comparative volt-ampere characteristics of the prior and present nonlinear resistance materials. In the graph, in which the volts and amperes are plotted in logarithmic scale, Curve B represents the prior material as made by the process described in the aforementioned Pitha patent, while Curve A represents resistance material of the present invention. As is evident, at the lower voltage levels, e.g., below 1,000 volts, the material represented by Curve A exhibits substantially higher resistivity than the Curve B material, while at voltages from 2,000 volts and higher, the resistivities of the respective materials are equivalent, and thus they provide equivalent protection under high overvoltage conditions. The increased resistivity of the improved resistance material at the lower voltage levels as shown is as much as 58 percent in terms of voltage required for passage of 1 ampere of current.

In a typical process of making the improved resistance material the following preferred composition in percent by weight has been found to produce satisfactory results for use in DC lightning arresters:

|                   |     |
|-------------------|-----|
| Silicon carbide   | 75% |
| Cordierite glass  | 10% |
| Talc              | 6%  |
| Porcelain mixture | 9%  |

As well understood by those versed in the art, the porcelain mixture may comprise flint, clay and soda or potash spar, but any particular type or composition of porcelain mixture may be utilized in practicing the present invention.

The cordierite glass used in the above mixture is made by mixing the following ingredients in the typical composition shown in percent by weight:

|                         |        |
|-------------------------|--------|
| $\text{SiO}_2$          | 51.3%  |
| $\text{Al}_2\text{O}_3$ | 34.9%  |
| $\text{MgO}$            | 13.8 % |

This mixture is heated to fusion in an electric arc furnace at a temperature no lower than about 1,800° C. causing the reaction of the ingredients and forming a molten glass material which is then quenched to prevent devitrification, as a result of which the material solidifies as a glass. The solid glass is thereafter ground into finely divided form for use in the binder mixture described above. When such glass is fired at elevated temperature below the melting point of the glass and thereafter cooled, it devitrifies (crystallizes) into a hard, dense ceramic material consisting of cordierite, which has the formula  $2\text{MgO} \cdot 2\text{Al}_2\text{O}_3 \cdot 5\text{SiO}_2$ .

The remaining binder ingredients, viz, talc and porcelain mixture, are also capable of forming cordierite when heated to

elevated temperature, but in contrast to the prereacted cordierite-forming glass component, are crystalline in nature and are employed in this form in the prefired mixture.

After all of the described components in finely divided form are mixed together and a suitable temporary binder such as water is added, the mixture is pressed into discs or otherwise formed into desired shapes, and in such form the material is fired at a temperature of from about 1,200° C. to about 1,300° C. in a hydrogen atmosphere, removed from the furnace and cooled. As a result of such firing and cooling, both the prereacted glass material and the crystalline binder ingredients form a ceramic binder composed of cordierite in crystalline form, with the silicon carbide particles held therein. As will be understood, the cooling of the fired material is relatively gradual, in distinction to the quenching step herein above referred to in connection with making the cordierite glass.

While the above specific composition is a typically preferred mixture, the resistance material of the invention may be formed from a composition within the following ranges, in percent by weight:

|                   |               |
|-------------------|---------------|
| Silicon carbide   | 55.0 to 80.0% |
| Cordierite glass  | 6.0 to 22.5%  |
| Talc              | 4.0 to 27.0%  |
| Porcelain mixture | 4.0 to 19.0 % |

An example of a suitable porcelain mixture which may be employed in the foregoing compositions is as follows, in percent by weight:

|                     |        |
|---------------------|--------|
| Flint               | 14.3%  |
| Clay                | 47.6%  |
| Soda or potash spar | 38.1 % |

Preferably, the talc and porcelain mixture components of the crystalline binder material vary in the range of 40 to 60 percent by weight of talc and 60 to 40 percent of porcelain mixture.

The porcelain mixture may be replaced by a china clay such as Florida kaolin, and in the binder mixture equal parts by weight of such kaolin and talc may typically be used as the cordierite-forming crystalline ingredients.

While the present invention has been described with reference to particular embodiments thereof, it will be understood that numerous modifications may be made by those

skilled in the art without actually departing from the scope of the invention. Therefore, the appended claims are intended to cover all such equivalent variations as come within the true spirit and scope of the invention.

5 What I claim as new and desire to secure by letters Patent of the United States is:

1. A composition for making nonlinear resistance material consisting essentially of a mixture of silicon carbide particles with a binder material having a composition comprising a mixture of cordierite-forming glass material and cordierite-forming crystalline material.

2. A composition as defined in claim 1, said composition consisting essentially of, in percent by weight, about 6.0 to about 22.5 percent of said glass material, about 8.0 to about 15 46.0 percent of said crystalline material, and about 55.0 to about 80.0 percent of said silicon carbide particles.

3. A composition as defined in claim 2, said crystalline material consisting essentially of, in percent by weight, about 40 to about 60 percent talc and about 60 to about 40 percent porcelain mixture.

4. A method of making nonlinear resistance material comprising the steps of providing a mixture as defined in claim 1, firing said mixture at elevated temperature for reacting said crystalline material, and cooling the thus-fired mixture for forming a cordierite binder for said silicon carbide particles from said mixture of glass material and crystalline material.

5. A method as defined in claim 4, including the step of compacting said mixture of silicon carbide particles and said cordierite-forming material prior to said firing step.

30 6. A method as defined in claim 5, said elevated temperature being in the range of about 1,200° C. to about 1,300° C.

7. A method as defined in claim 6, said compacted mixture being fired in a hydrogen atmosphere.

8. A nonlinear resistance material having improved low voltage resistance characteristics coupled with a high capacity for withstanding repeated current surges for use in overvoltage protective devices, said material being made by the process defined in claim 4.

9. A nonlinear resistance material having improved low voltage resistance characteristics coupled with a high capacity for withstanding repeated current surges for use in overvoltage protective devices, said material being made by the process defined in claim 6.

UNITED STATES PATENT OFFICE  
CERTIFICATE OF CORRECTION

Patent No. 3,607,790 Dated September 21, 1971

Inventor(s) John J. Pitha

It is certified that error appears in the above-identified patent and that said Letters Patent are hereby corrected as shown below:

Col. 1, line 35, after "resistivity" insert -  
characteristics for passing current  
during overvoltage -

" " line 43, correct the spelling of "cordierite"  
Signed and sealed this 29th day of February 1972.

(SEAL)

Attest:

EDWARD M. FLETCHER, JR.  
Attesting Officer

ROBERT GOTTSCHALK  
Commissioner of Patents